# EUROPEAN PATENT SPECIFICATION

(11) **EP 2 325 343 B1**
(45) Date of publication and mention of the grant of the patent: **25.12.2013**
(21) Application number: 10251470.0
(22) Date of filing: 19.08.2010
(51) Int. Cl.: C22C 1/04, C22C 21/00, C22F 1/04, B22F 1/00, B22F 3/12, B22F 3/14, B22F 3/17, B22F 3/20

(54) **Forging deformation of L12 aluminum alloys**
Schmiedeverformung von L12-Aluminiumlegierungen
Déformation au forgeage d'alliages d'aluminium L12

(30) Priority: 16.10.2009 US 589105
(43) Date of publication of application: 25.05.2011
(73) Proprietor: United Technologies Corporation, Hartford, CT 06101 (US)
(72) Inventor: Pandey, Awadh B., Jupiter Florida 33458 (US)
(74) Representative: Hall, Matthew Benjamin

(56) References cited:
- EP-A2- 1 111 078
- WO-A2-03/104505
- US-A- 5 226 983

## Description

The present invention relates generally to aluminum alloys and more specifically to a method for forming high strength aluminum alloy powder having L1₂ dispersoids therein into useful parts.

The combination of high strength, ductility, and fracture toughness, as well as low density, make aluminum alloys natural candidates for as variety of applications. Because of its low weight high strength, ductility and fracture toughness, aluminum alloys are of interest in the manufacture and use for many applications.

The development of aluminum alloys with improved elevated temperature mechanical properties is a continuing process. Some attempts have included aluminum-iron and aluminum-chromium based alloys such as Al-Fe-Ce, Al-Fe-V-Si, Al-Fe-Ce-W, and Al-Cr-Zr-Mn that contain incoherent dispersoids. These alloys, however, also lose strength at elevated temperatures due to particle coarsening. In addition, these alloys exhibit ductility and fracture toughness values lower than other commercially available aluminum alloys.

Other attempts have included the development of mechanically alloyed Al-Mg and Al-Ti alloys containing ceramic dispersoids. These alloys exhibit improved high temperature strength due to the particle dispersion, but the ductility and fracture toughness are not improved.

U.S. patent 6,248,453 discloses aluminum alloys strengthened by dispersed Al₃X L1₂ intermetallic phases where X is selected from the group consisting of Sc, Er, Lu, Yb, Tm, and Lu. The A1₃X particles are coherent with the aluminum alloy matrix and are resistant to coarsening at elevated temperatures. The improved mechanical properties of the disclosed dispersion strengthened L1₂ aluminum alloys are stable up to 572°F (300°C). U.S. Patent Application Publication No. 2006/0269437 A1 discloses a high strength aluminum alloy that contains scandium and other elements that is strengthened by L1₂ dispersoids.

L1₂ strengthened aluminum alloys have high strength and improved fatigue properties compared to commercial aluminum alloys. Fine grain size results in improved mechanical properties of materials. Hall-Petch strengthening has been known for decades where strength increases as grain size decreases. An optimum grain size for optimum strength is in the nano range of about 30 to 100 nm. These alloys also have higher ductility.

The present invention is a method for consolidating aluminum alloy powders into useful components having improved strength and fracture toughness.

The aluminum alloy parts are formed by isothermal forging of consolidated billets. Isothermal forging of these alloys produces considerable improvement in mechanical properties, especially ductility compared to the consolidated billet. Forging parameters include billet temperature, billet soak time, forging rate, reduction and die temperature.

According to one aspect of the present invention there is provided a method according to claim 1.

According to one other aspect of the present invention there is provided a high strength aluminum alloy component according to claim 5.

Certain preferred embodiments will now be described, by way of example only, with reference to the accompanying drawings.
FIG. 1 is an aluminum scandium phase diagram.
FIG. 2A is a schematic diagram of a vertical gas atomizer.
FIG. 2B is a close up view of nozzle 108 in FIG. 2A.
FIG. 3A and 3B are SEM photos of the inventive aluminum alloy powder.
FIG. 4A and 4B are optical micrographs showing the microstructure of gas atomized L1₂ aluminum alloy powder.
FIG. 5 is a diagram showing the steps of the gas atomization process.
FIG. 6 is a diagram showing the processing steps to consolidate the L1₂ aluminum alloy powder.
FIG. 7 is a schematic diagram of blind die compaction.
FIG. 8 is a schematic diagram of a forging process.
FIG. 9A is a photo of a L1₂ aluminum alloy pancake forging.
FIG. 9B and 9C are photos of an L1₂ aluminum alloy turbine rotor.

### 1. L1₂ Aluminum Alloys

Alloy powders of this invention are formed from aluminum based alloys with high strength and fracture toughness for applications at temperatures from about -420°F (-251°C) up to about 650°F (343°C). The aluminum alloy is strengthened by L1₂ Al₃X coherent precipitates the aluminum alloy having the composition Al-5.0Cu-1.5Mg-1.0Li-0.45Sc-0.21Nb-0.2Zr (wt%).

The binary aluminum magnesium system is a simple eutectic at 36 weight percent magnesium and 842°F (450°C). There is complete solubility of magnesium and aluminum in the rapidly solidified inventive alloys discussed herein.

The binary aluminum lithium system is a simple eutectic at 8 weight percent lithium and 1105° (596°C). The equilibrium solubility of 4 weight percent lithium can be extended significantly by rapid solidification techniques. There is complete solubility of lithium in the rapid solidified inventive alloys discussed herein.

The binary aluminum copper system is a simple eutectic at 32 weight percent copper and 1018°F (548°C). There is complete solubility of copper in the rapidly solidified inventive alloys discussed herein.

In the aluminum based alloy, scandium is a potent strengthener that has low diffusivity and low solubility in aluminum. This element forms equilibrium Al₃X intermetallic dispersoids where X is scandium, that have an L1₂ structure that is an ordered face centered cubic structure with the X atoms located at the corners and aluminum atoms located on the cube faces of the unit cell.

Scandium forms Al₃Sc dispersoids that are fine and coherent with the aluminum matrix. Lattice parameters of aluminum and Al₃Sc are very close (0.405 nm and 0.410 nm respectively), indicating that there is minimal or no driving force for causing growth of the Al₃Sc dispersoids. This low interfacial energy makes the Al₃Sc dispersoids thermally stable and resistant to coarsening up to temperatures as high as about 842°F (450°C). Additions of magnesium in aluminum increase the lattice parameter of the aluminum matrix, and decrease the lattice parameter mismatch further increasing the resistance of the Al₃Sc to coarsening. Additions of copper and lithium provide solid solution and precipitation strengthening in the aluminum alloys. These Al₃Sc dispersoids are made stronger and more resistant to coarsening at elevated temperatures by adding suitable alloying elements such as zirconium and niobium that enter Al₃Sc in solution.

Zirconium forms Al₃Zr dispersoids in the aluminum matrix that have an L1₂ structure in the metastable condition and D0₂₃ structure in the equilibrium condition. The metastable Al₃Zr dispersoids have a low diffusion coefficient, which makes them thermally stable and highly resistant to coarsening. Zirconium has a high solubility in the Al₃X dispersoids allowing large amounts of zirconium to substitute for X in the Al₃X dispersoids, which results in improved thermal and structural stability.

Niobium forms metastable Al₃Nb dispersoids in the aluminum matrix that have an L1₂ structure in the metastable condition and a D0₂₂ structure in the equilibrium condition. Niobium has a lower solubility in the Al₃X dispersoids than hafnium or yttrium, allowing relatively lower amounts of niobium than hafnium or yttrium to substitute for X in the Al₃X dispersoids. Nonetheless, niobium can be very effective in slowing down the coarsening kinetics of the Al₃X dispersoids because the Al₃Nb dispersoids are thermally stable. The substitution of niobium for X in the above mentioned Al₃X dispersoids results in stronger and more thermally stable dispersoids.

Al₃X L1₂ precipitates improve elevated temperature mechanical properties in aluminum alloys for two reasons. First, the precipitates are ordered intermetallic compounds. As a result, when the particles are sheared by glide dislocations during deformation, the dislocations separate into two partial dislocations separated by an anti-phase boundary on the glide plane. The energy to create the anti-phase boundary is the origin of the strengthening. Second, the cubic L1₂ crystal structure and lattice parameter of the precipitates are closely matched to the aluminum solid solution matrix. This results in a lattice coherency at the precipitate/matrix boundary that resists coarsening. The lack of an interphase boundary results in a low driving force for particle growth and resulting elevated temperature stability. Alloying elements in solid solution in the dispersed strengthening particles and in the aluminum matrix that tend to decrease the lattice mismatch between the matrix and particles will tend to increase the strengthening and elevated temperature stability of the alloy.

L1₂ phase strengthened aluminum alloys are important structural materials because of their excellent mechanical properties and the stability of these properties at elevated temperature due to the resistance of the coherent dispersoids in the microstructure to particle coarsening. The mechanical properties are optimized by maintaining a high volume fraction of L1₂ dispersoids in the microstructure. The L1₂ dispersoid concentration following aging scales as the amount of L1₂ phase forming elements in solid solution in the aluminum alloy following quenching. Examples of L1₂ phase forming elements includes Sc. The concentration of alloying elements in solid solution in alloys cooled from the melt is directly proportional to the cooling rate.

The Al-Sc phase diagram shown in FIG. 1 indicates a eutectic reaction at about 0.5 weight percent scandium at about 1219°F (659°C) resulting in a solid solution of scandium and aluminum and Al₃Sc dispersoids. Aluminum alloys with less than 0.5 weight percent scandium can be quenched from the melt to retain scandium in solid solution that may precipitate as dispersed L1₂ intermetallic Al₃Sc following an aging treatment. Alloys with scandium in excess of the eutectic composition (hypereutectic alloys) can only retain scandium in solid solution by rapid solidification processing (RSP) where cooling rates are in excess of about 10³°C/second.

### 2. L1₂ Alloy Powder Formation and Consolidation

The highest cooling rates observed in commercially viable processes are achieved by gas atomization of molten metals to produce powder. Gas atomization is a two fluid process wherein a stream of molten metal is disintegrated by a high velocity gas stream. The end result is that the particles of molten metal eventually become spherical due to surface tension and finely solidify in powder form. Heat from the liquid droplets is transferred to the atomization gas by convection. The solidification rates, depending on the gas and the surrounding environment, can be very high and can exceed 10⁶°C/second. Cooling rates greater than 10³°C/second are typically specified to ensure supersaturation of alloying elements in gas atomized L1₂ aluminum alloy powder in the inventive process described herein.

A schematic of typical vertical gas atomizer 100 is shown in FIG. 2A. FIG. 2A is taken from R. Germain, Powder Metallurgy Science Second Edition MPIF (1994) (chapter 3, p. 101) and is included herein for reference. Vacuum or inert gas induction melter 102 is positioned at the top of free flight chamber 104. Vacuum induction melter 102 contains melt 106 which flows by gravity or gas overpressure through nozzle 108. A close up view of nozzle 108 is shown in FIG. 2B. Melt 106 enters nozzle 108 and flows downward till it meets the high pressure gas stream from gas source 110 where it is transformed into a spray of droplets. The droplets eventually become spherical due to surface tension and rapidly solidify into spherical powder 112 which collects in collection chamber 114. The gas recirculates through cyclone collector 116 which collects fine powder 118 before returning to the input gas stream. As can be seen from FIG. 2A, the surroundings to which the melt and eventual powder are exposed are completely controlled.

There are many effective nozzle designs known in the art to produce spherical metal powder. Designs with short gas-to-melt separation distances produce finer powders. Confined nozzle designs where gas meets the molten stream at a short distance just after it leaves the atomization nozzle are preferred for the production of the inventive L1₂ aluminum alloy powders. Higher superheat temperatures cause lower melt viscosity and longer cooling times. Both result in smaller spherical particles.

A large number of processing parameters are associated with gas atomization that affect the final product. Examples include melt superheat, gas pressure, metal flow rate, gas type, and gas purity. In gas atomization, the particle size is related to the energy input to the metal. Higher gas pressures, higher superheat temperatures and lower metal flow rates result in smaller particle sizes. Higher gas pressures provide higher gas velocities for a given atomization nozzle design.

To maintain purity, inert gases are used, such as helium, argon, and nitrogen. Helium is preferred for rapid solidification because the high heat transfer coefficient of the gas leads to high quenching rates and high supersaturation of alloying elements.

Lower metal flow rates and higher gas flow ratios favor production of finer powders. The particle size of gas atomized melts typically has a log normal distribution. In the turbulent conditions existing at the gas/metal interface during atomization, ultra fine particles can form that may reenter the gas expansion zone. These solidified fine particles can be carried into the flight path of molten larger droplets resulting in agglomeration of small satellite particles on the surfaces of larger particles. An example of small satellite particles attached to inventive spherical L1₂ aluminum alloy powder is shown in the scanning electron microscopy (SEM) micrographs of FIG. 7A and 7B at two magnifications. The spherical shape of gas atomized aluminum powder is evident. The spherical shape of the powder is suggestive of clean powder without excessive oxidation. Higher oxygen in the powder results in irregular powder shape. Spherical powder helps in improving the flowability of powder which results in higher apparent density and tap density of the powder. The satellite particles can be minimized by adjusting processing parameters to reduce or even eliminate turbulence in the gas atomization process. The microstructure of gas atomized aluminum alloy powder is predominantly cellular as shown in the optical micrographs of cross-sections of the inventive alloy in FIG. 8A and 8B at two magnifications. The rapid cooling rate suppresses dendritic solidification common at slower cooling rates resulting in a finer microstructure with minimum alloy segregation.

Oxygen and hydrogen in the powder can degrade the mechanical properties of the final part. It is preferred to limit the oxygen in the L1₂ alloy powder to about 1 ppm to 2000 ppm. Oxygen is intentionally introduced as a component of the helium gas during atomization. An oxide coating on the L1₂ aluminum powder is beneficial for two reasons. First, the coating prevents agglomeration by contact sintering and secondly, the coating inhibits the chance of explosion of the powder. A controlled amount of oxygen is important in order to provide good ductility and fracture toughness in the final consolidated material. Hydrogen content in the powder is controlled by ensuring the dew point of the helium gas is low. A dew point of about minus 50°F (minus 45.5°C) to minus 100°F (minus 73.3°C) is preferred.

In preparation for final processing, the powder is classified according to size by sieving. To prepare the powder for sieving, if the powder has zero percent oxygen content, the powder may be exposed to nitrogen gas which passivates the powder surface and prevents agglomeration. Finer powder sizes result in improved mechanical properties of the end product. While minus 325 mesh (about 45 microns) powder can be used, minus 450 mesh (about 30 microns) powder is a preferred size in order to provide good mechanical properties in the end product. During the atomization process, powder is collected in collection chambers in order to prevent oxidation of the powder. Collection chambers are used at the bottom of atomization chamber 104 as well as at the bottom of cyclone collector 116. The powder is transported and stored in the collection chambers also. Collection chambers are maintained under positive pressure with nitrogen gas which prevents oxidation of the powder.

A schematic of the L1₂ aluminum powder manufacturing process is shown in FIG. 9. In the process aluminum 200 and L1₂ forming (and other alloying) elements 210 are melted in furnace 220 to a predetermined superheat temperature under vacuum or inert atmosphere. Preferred charge for furnace 220 is prealloyed aluminum 200 and L1₂ and other alloying elements before charging furnace 220. Melt 230 is then passed through nozzle 240 where it is impacted by pressurized gas stream 250. Gas stream 250 is an inert gas such as nitrogen, argon or helium, preferably helium. Melt 230 can flow through nozzle 240 under gravity or under pressure. Gravity flow is preferred for the inventive process disclosed herein. Preferred pressures for pressurized gas stream 250 are about 50 psi (10.35 MPa) to about 750 psi (5.17 MPa) depending on the alloy.

The atomization process creates molten droplets 260 which rapidly solidify as they travel through agglomeration chamber 270 forming spherical powder particles 280. The molten droplets transfer heat to the atomizing gas by convention. The role of the atomizing gas is two fold: one is to disintegrate the molten metal stream into fine droplets by transferring kinetic energy from the gas to the melt stream and the other is to extract heat from the molten droplets to rapidly solidify them into spherical powder. The solidification time and cooling rate vary with droplet size. Larger droplets take longer to solidify and their resulting cooling rate is lower. On the other hand, the atomizing gas will extract heat efficiently from smaller droplets resulting in a higher cooling rate. Finer powder size is therefore preferred as higher cooling rates provide finer microstructures and higher mechanical properties in the end product. Higher cooling rates lead to finer cellular microstructures which are preferred for higher mechanical properties. Finer cellular microstructures result in finer grain sizes in consolidated product. Finer grain size provides higher yield strength of the material through the Hall-Petch strengthening model.

Key process variables for gas atomization include superheat temperature, nozzle diameter, helium content and dew point of the gas, and metal flow rate. Superheat temperatures of from about 150°F (66°C) to 200°F (93°C) are preferred. Nozzle diameters of about 0.07 in. (1.8 mm) to 0.12 in. (3.0 mm) are preferred depending on the alloy. The gas stream used herein was a helium nitrogen mixture containing 74 to 87 vol. % helium. The metal flow rate ranged from about 0.8 1b/min (0.36 kg/min) to 4.0 1b/min (1.81 kg/min). The oxygen content of the L1₂ aluminum alloy powders was observed to consistently decrease as a run progressed. This is suggested to be the result of the oxygen gettering capability of the aluminum powder in a closed system. The dew point of the gas was controlled to minimize hydrogen content of the powder. Dew points in the gases used in the examples ranged from - 10°F (-23°C) to -110°F (-79°C).

The powder is then classified by sieving process 290 to create classified powder 300. Sieving of powder is performed under an inert environment to minimize oxygen and hydrogen pickup from the environment. While the yield of minus 450 mesh (30 µm) powder is extremely high (95%), there are always larger particle sizes, flakes and ligaments that are removed by the sieving. Sieving also ensures a narrow size distribution and provides a more uniform powder size. Sieving also ensures that flaw sizes cannot be greater than minus 450 mesh (30 µm) which will be required for nondestructive inspection of the final product.

Processing parameters of exemplary gas atomization runs are listed in Table 1.

**Table 1: Gas atomization parameters used for producing powder**

| Run | Nozzle Diameter in (cm) | He Content (vol%) | Gas Pressure psi (MPa) | Dew Point °F (°C) | Charge Temperature °F (°C) | Average Metal Flow Rate lbs/min (kg/min) | Oxygen Content (ppm) Start | Oxygen Content (ppm) End |
|---|---|---|---|---|---|---|---|---|
| 1 | 0.10 (0.25) | 79 | 190 (1.31) | <-58 (-50) | 2200 (1204) | 2.8 (1.27) | 340 | 35 |
| 2 | 0.10 (0.25) | 83 | 192 (1.32) | -35 (-37) | 1635 (891) | 0.8 (.36) | 772 | 27 |
| 3 | 0.09 (0.25) | 78 | 190 (1.31) | -10 (-23) | 2230 (1221) | 1.4 (.64) | 297 | <0.01 |
| 4 | 0.09 (0.25) | 85 | 160 (1.10) | -38 (-39) | 1845 (1007) | 2.2 (1.0) | 22 | 4.1 |
| 5 | 0.10 (0.25) | 86 | 207 (1.43) | -88 (-67) | 1885 (1029) | 3.3 (1.5) | 286 | 208 |
| 6 | 0.09 (0.25) | 86 | 207 (1.43) | -92 (-69) | 1915 (1046) | 2.6 (1.2) | 145 | 88 |

The role of powder quality is extremely important to produce material with higher strength and ductility. Powder quality is determined by powder size, shape, size distribution, oxygen content, hydrogen content, and alloy chemistry. Over fifty gas atomization runs were performed to produce the inventive powder with finer powder size, finer size distribution, spherical shape, and lower oxygen and hydrogen contents. Processing parameters of some exemplary gas atomization runs are listed in Table 1. It is suggested that the observed decrease in oxygen content is attributed to oxygen gettering by the powder as the runs progressed.

Inventive L1₂ aluminum alloy powder was produced with over 95% yield of minus 450 mesh (30 microns) which includes powder from about 1 micron to about 30 microns. The average powder size was about 10 microns to about 15 microns. As noted above, finer powder size is preferred for higher mechanical properties. Finer powders have finer cellular microstructures. As a result, finer cell sizes lead to finer grain size by fragmentation and coalescence of cells during powder consolidation. Finer grain sizes produce higher yield strength through the Hall-Petch strengthening model where yield strength varies inversely as the square root of the grain size. It is preferred to use powder with an average particle size of 10-15 microns. Powders with a powder size less than 10-15 microns can be more challenging to handle due to the larger surface area of the powder. Powders with sizes larger than 10-15 microns will result in larger cell sizes in the consolidated product which, in turn, will lead to larger grain sizes and lower yield strengths.

Powders with narrow size distributions are preferred. Narrower powder size distributings produce product microstructures with more uniform grain size. Spherical powder was produced to provide higher apparent and tap densities which help in achieving 100% density in the consolidated product. Spherical shape is also an indication of cleaner and lower oxygen content powder. Lower oxygen and lower hydrogen contents are important in producing material with high ductility and fracture toughness. Although it is beneficial to maintain low oxygen and hydrogen content in powder to achieve good mechanical properties, lower oxygen may interfere with sieving due to self sintering. An oxygen content of about 25 ppm to about 500 ppm is preferred to provide good ductility and fracture toughness without any sieving issue. Lower hydrogen is also preferred for improving ductility and fracture toughness. It is preferred to have about 25-200 ppm of hydrogen in atomized powder by controlling the dew point in the atomization chamber. Hydrogen in the powder is further reduced by heating the powder in vacuum. Lower hydrogen in final product is preferred to achieve good ductility and fracture toughness.

A schematic of the L1₂ aluminum powder consolidation process is shown in FIG. 6. The starting material is sieved and classified L1₂ aluminum alloy powders (step 310). Blending (step 320) is a preferred step in the consolidation process because it results in improved uniformity of particle size distribution. Gas atomized L1₂ aluminum alloy powder generally exhibits a bimodal particle size distribution and cross blending of separate powder batches tends to homogenize the particle size distribution. Blending (step 320) is also preferred when separate metal and/or ceramic powders are added to the L1₂ base powder to form bimodal or trimodal consolidated alloy microstructures.

Following blending (step 320), the powders are transferred to a can (step 330) where the powder is vacuum degassed (step 340) at elevated temperatures. The can (step 330) is an aluminum container having a cylindrical, rectangular or other configuration with a central axis. Cylindrical configurations are preferred with hydraulic extrusion presses. Vacuum degassing times can range from about 0.5 hours to about 8 days. A temperature range of about 300°F (149°C) to about 900°F (482°C) is preferred. Dynamic degassing of large amounts of powder is preferred to static degassing. In dynamic degassing, the can is preferably rotated during degassing to expose all of the powder to a uniform temperature. Degassing removes oxygen and hydrogen from the powder.

Following vacuum degassing (step 340), the vacuum line is crimped and welded shut (step 350). The powder is then fully densified by blind die compaction or closed die forging as the process is sometimes called (step 360). At this point the can may be removed by machining (step 380) to form a useful billet (step 390).

A schematic showing blind die compaction (process 400) is shown in FIGS. 7A and 7B. The equipment comprises base 410, die 420, ram 430, and means to apply pressure to ram 430 indicated by arrow 450. Prior to compaction, billet 440 does not fill die cavity 460. After compaction, billet 445 completely fills the die cavity and has taken the shape of die cavity 460. The die cavities can have any shape provided they have a central symmetrical axis parallel to arrow 450. Cylindrical shapes adopt well for extrusion billets. Canned L1₂ aluminum alloy powder preforms are easily densified due to the large capacity of modern hydraulic presses.

### 3. Forging of L1₂ Consolidated Alloys

Conventional Forging such as drop and hammer forging is performed at high strain rates where adiabatic heating may result in loss of strength due to microstructural coarsening. Isothermal forging at moderate to low strain rates offers the same microstructural refinement due to forging deformation but eliminates the chance for adiabatic heating. Forging can be with or without a die depending on the required forged billet shape using conventional forging or isothermal forging.

A schematic sketch of forging operation 500 is shown in FIG. 8. Forging operation 500 comprises bottom die 510, upper die 520, and press mechanism 540. During forging, press mechanism 540 applies pressure P to upper die 520 and moves movable upper die 520 toward billet 530 along axis 545 and compresses billet 540 decreasing the thickness of billet 540 and impressing the features of bottom die face 515 and upper die face 525 on billet 530. This type of forging is termed open die or pancake forging wherein billet 540 expands radially in all directions in the absence of any constraints. If bottom die 510 contained vertical constraints (walls) 550 that limit the deformation of billet 530 to a constant volume defined by walls 550, forging operation 500 is termed closed die forging. It is to be understood that bottom die 510 could be a moveable die attached to press mechanism 540 and upper die 520 could be a fixed die. Press mechanism 540 is commonly a hydraulic mechanism because of the capacity of modem hydraulic presses.

Consolidated L1₂ alloy powder can be directly forged but the mechanical properties are inferior to consolidated powder that has been extruded before forging. In the example discussed herein, the starting workpieces were consolidated L1₂ powders in aluminum cans. The cans were removed by machining and the billets were extruded through a rectangular die to produce billets with rectangular cross sections that were then isothermally vacuum forged in a hydraulic press with heated platens. Forging parameters that result in L1₂ alloys with improved mechanical properties have been developed and are discussed here. Forging parameters include billet temperature, billet soak time, forging rate, reduction and temperature. All forging results were obtained by open die pancake forging.

Table 2 shows the effect of forging parameters on tensile properties of an Al-5.0Cu-1.5Mg-1.0Li-0.45Sc-0.21Nb-0.2Zr (all in wt%) alloy. Forging temperature was varied from 475°F (246°C) to 650°F (243°C), strain rate varied from 0.1 to 0.4 inch per minute and deformation was maintained constant at about 85% for these examples. Yield strengths of 103-106 ksi (710-731 MPa), tensile strengths of 108-114 ksi (745-786 MPa) and elongations of 9-12 percent were observed for this alloy.

**Table 2: Al-5.0Cu-1.5Mg-1.0Li-0.45Sc-0.21Nb-0.2Zr alloy**

| Sample ID | Forging Temperature, °F (°C) | Strain Rate, inch/min (mm/min) | Deformation, % | Yield Strength, ksi (MPa) | Tensile Strength, ksi (MPa) | Elongation, % |
|---|---|---|---|---|---|---|
| 1 | 650 (343) | 0.1 (2.5) | 86 | 102.5 (707) | 110 (758) | 9.5 |
| 2 | 650 (343) | 0.1 (2.5) | 86 | 104 (717) | 111 (756) | 9 |
| 3 | 475 (246) | 0.1 (2.5) | 85 | 105 (724) | 112 (772) | 11 |
| 4 | 475 (246) | 0.4 (10.2) | 84 | 103.5 (714) | 108 (745) | 11.4 |
| 5 | 475 (246) | 0.4 (10.2) | 84 | 106 (731) | 112 (776) | 12 |
| 6 | 475 (246) | 0.4 (10.2) | 85 | 105.5(736) | 114 (786) | 10.5 |

## Claims

1. A method for forming a high strength aluminum alloy component containing L1₂ dispersoids, comprising the steps of:
placing in a container a quantity of an aluminum alloy powder containing an L1₂ dispersoid L1₂ comprising Al₃X dispersoids wherein the composition of the powder is Al-5.0Cu-1.5Mg-1.0Li-0.45Sc-0.21Nb-0.2Zr (in wt%);
vacuum degassing the powder at a temperature of 300°F (149°C) to 900°F (482°C) for 0.5 hours to 8 days;
sealing the degassed powder in the container under vacuum;
heating the sealed container at 300°F (149°C) to 900°F (482°C) for 15 minutes to eight hours;
vacuum hot pressing the heated container to form a billet;
removing the container from the formed billet; and
forging the billet into a component with improved strength and fracture toughness, wherein the forging temperature is between 475°F (246°C) to 650°F (243°C), the strain rate is between 0.1 to 0.4 inch per minute (2.54 to 10.16 mm/min) and the deformation is about 85%,
wherein the tensile strength of forged L1₂ alloy billet is from 108 ksi (745 MPa) to 114 ksi (786 MPa), wherein the yield strength of forged L1₂ alloy billet is from 103 ksi (710 MPa) to 106 ksi (731 MPa) and wherein the elongation of forged L1₂ alloy billet is from 9 to 12 percent.

2. The method of claim 1, wherein the alloy powder has a mesh size of less than 350 mesh (42 µm).

3. A high strength aluminum alloy component, comprising:
an aluminum alloy billet containing an L1₂ dispersoid comprising Al₃X dispersoids wherein the composition of the aluminum alloy is Al-5.0Cu-1.5Mg-1.0Li-0.45Sc-0.21Nb-0.2Zr (wt%),
the billet being forged into a component with improved strength and fracture toughness, wherein the forging temperature is between 475°F (246°C) to 650°F (243°C), the strain rate is between 0.1 to 0.4 inch per minute (2.54 to 10.16 mm/min) and the deformation is about 85%,
wherein the tensile strength of forged L1₂ alloy billet is from 108 ksi (745 MPa) to 114 ksi (786 MPa)
wherein the yield strength of forged alloy billet is from 103 ksi (710 MPa) to 106 ksi (731 MPa), and,
wherein the elongation of forged L1₂ alloy billet is from 9 to 12 percent.

4. The alloy component of claim 3, wherein the alloy powder has a mesh size of less than 350 mesh (42 µm).

## Patentansprüche

1. Verfahren zur Herstellung einer Komponente aus einer hochfesten Aluminiumlegierung, die L1₂-Dispersoide enthält, folgende Schritte aufweisend:
Einbringen einer Menge eines Aluminiumlegierungspulvers, das ein Al₃X-Dispersoide aufweisendes L1₂-Dispersoid L1₂ enthält, wobei die Zusammensetzung des Pulvers (in Gew%) Al-5, 0Cu-1,5Mg-1, 0Li-0, 45Sc-0, 21Nb-0, 2Zr ist, in einen Behälter;
Entgasen des Pulvers unter Vakuum bei einer Temperatur von 300° F (149° C) bis 900° F (482° C) für 0,5 Stunden bis 8 Tage;
dicht Einschließen des entgasten Pulvers in dem Behälter unter Vakuum;
Erhitzen des dicht verschlossenen Behälters bei 300° F (149° C) bis 900° F (482° C) für 15 Minuten bis 8 Stunden;
Heißpressen des erhitzten Behälters unter Vakuum, um einen Block zu bilden;
Entfernen des Behälters von dem gebildeten Block; und
Schmieden des Blocks zu einer Komponente mit verbesserter Festigkeit und Bruchzähigkeit, wobei die Schmiedetemperatur zwischen 475° F (246° C) bis 650° F (243° C) liegt, die Verformungsgeschwindigkeit zwischen 0,1 bis 0,4 Zoll pro Minute (2,54 bis 10,16 mm/min) liegt, und die Verformung etwa 85% beträgt,
wobei die Zerreißfestigkeit eines geschmiedeten L1₂-Legierungsblocks von 108 ksi (745 MPa) bis 114 ksi (786 MPa) beträgt, wobei die Streckgrenze eines geschmiedeten L1₂-Legierungsblocks von 103 ksi (710 MPa) bis 106 ksi (731 MPa) beträgt, und wobei die Dehnung eines geschmiedeten L1₂-Legierungsblocks von 9 bis 12 Prozent beträgt.

2. Verfahren nach Anspruch 1, wobei das Legierungspulver eine Maschengröße von weniger als 350 Mesch (42 µm) hat.

3. Komponente aus hochfester Aluminiumlegierung, aufweisend:
einen Block aus Aluminiumlegierung, die ein Al₃X-Dispersoide aufweisendes L1₂-Dispersoid enthält, wobei die Zusammensetzung der Aluminiumlegierung Al-5, 0Cu-1, 5Mg-1, 0Li-0, 45Sc-0, 21Nb-0, 2Zr (Gew%) ist,
wobei der Block zu einer Komponente mit verbesserter Festigkeit und Bruchzähigkeit geschmiedet wird, wobei die Schmiedetemperatur zwischen 475° F (246° C) bis 650° F (243° C) liegt, die Verformungsgeschwindigkeit zwischen 0,1 bis 0,4 Zoll pro Minute (2,54 bis 10,16 mm/min) liegt und die Verformung etwa 85% beträgt,
wobei die Zerreißfestigkeit eines geschmiedeten L1₂-Legierungsblocks von 108 ksi (745 MPa) bis 114 ksi (186 MPa) beträgt,
wobei die Streckgrenze eines geschmiedeten Legierungsblocks von 103 ksi (710 MPa) bis 106 ksi (731 MPa) beträgt, und
wobei die Dehnung eines geschmiedeten L1₂-Legierungsblocks von 9 bis 12 Prozent beträgt.

4. Legierungskomponente nach Anspruch 3, wobei das Legierungspulver eine Maschengröße von weniger als 350 Mesch (42 µm) hat.

## Revendications

1. Procédé de formation d'un composant d'alliage d'aluminium de résistance élevée contenant des dispersoïdes de L1₂, comprenant les étapes consistant à :
placer dans un conteneur une quantité d'une poudre d'alliage d'aluminium contenant un dispersoïde de L1₂ comprenant des dispersoïdes d'Al₃X, dans lequel la composition de la poudre est la suivante : Al - 5,0 0 Cu - 1,5 Mg - 1,0 Li - 0,45 Sc - 0,21 Nb - 0,2 Zr (en % en poids) ;
dégazer sous vide la poudre à une température de 300 °F (149 °C) à 900 °F (482 °C) sur une période de 0,5 heure à 8 jours ;
sceller la poudre dégazée dans le conteneur sous vide ;
chauffer le conteneur scellé à une température de 300 °F (149 °C) à 900 °F (482 °C) sur une période de 15 minutes à 8 heures ;
comprimer à chaud sous vide le conteneur chauffé pour former une billette ;
retirer le conteneur de la billette formée ; et
forger la billette pour en faire un composant de plus grande résistance et de plus forte ténacité à la rupture, dans lequel la température de forgeage se situe entre 475 °F (246 °C) et 650 °F (243 °C), le taux de déformation se situe entre 0,1 et 0,4 pouce par minute (2,54 à 10,16 mm/min) et la déformation est d'environ 85 %,
dans lequel la résistance à la traction de la billette d'alliage de Ll₂ forgée est de 108 ksi (745 MPa) à 114 ksi (786 MPa), dans lequel la résistance à la déformation de la billette d'alliage de L1₂ forgée est de 103 ksi (710 MPa) à 106 ksi (731 MPa) et dans lequel l'allongement de la billette d'alliage de L1₂ forgée est de 9 à 12 pour cent.

2. Procédé selon la revendication 1, dans lequel la poudre d'alliage présente une taille granulométrique inférieure à 350 mesh (42 µm).

3. Composant d'alliage d'aluminium de résistance élevée, comprenant :
une billette d'alliage d'aluminium contenant un dispersoïde de Ll₂ comprenant des dispersoïdes d'Al₃X, dans lequel la composition de l'alliage d'aluminium est la suivante : Al - 5,0 Cu - 1,5 Mg - 1,0 Li - 0,45 Sc - 0,21 Nb - 0,2 Zr (en % en poids) ;
la billette étant forgée pour en faire un composant de plus grande résistance et de plus forte ténacité à la rupture, dans lequel la température de forgeage se situe entre 475 °F (246 °C) et 650 °F (243 °C), le taux de déformation se situe entre 0,1 et 0,4 pouce par minute (2,54 à 10,16 mm/min) et la déformation est d'environ 85 %,
dans lequel la résistance à la traction de la billette d'alliage de L1₂ forgée est de 108 ksi (745 MPa) à 114 ksi (786 MPa),
dans lequel la résistance à la déformation de la billette d'alliage forgée est de 103 ksi (710 MPa) à 106 ksi (731 MPa) et
dans lequel l'allongement de la billette d'alliage de L1₂ forgée est de 9 à 12 pour cent.

4. Composant d'alliage selon la revendication 3, dans lequel la poudre d'alliage présente une taille granulométrique inférieure à 350 mesh (42 µm).
